

Patented Dec. 15, 1925.

## UNITED STATES PATENT OFFICE.

EDGAR CORNELL, JR., OF PITTSBURGH, PENNSYLVANIA, ASSIGNOR TO WESTINGHOUSE ELECTRIC & MANUFACTURING COMPANY, A CORPORATION OF PENNSYLVANIA.

## METHOD OF TREATING COATED MATERIALS.

No Drawing.

Application filed December 21, 1923. Serial No. 682,108.

To all whom it may concern:

Be it known that I, EDGAR CORNELL, Jr., a citizen of the United States, and a resident of Pittsburgh, in the county of Allegheny and State of Pennsylvania, have invented 5 a new and useful Improvement in Methods of Treating Coated Materials, of which the following is a specification.

This invention relates to coated materials, 10 more particularly to metal articles coated with zinc or the like.

Heretofore, it has been customary to coat metal articles, which are intended to be exposed to atmospheric conditions, with zinc or like materials by one of several processes, 15 such as electro-galvanizing, hot galvanizing or sherardizing. The zinc coating was brittle and had a tendency to peel or flake off, owing to the crystalline structure of the 20 zinc. This was the case regardless of the method of deposition of the coating, but ordinarily this defect was not detrimental to the article because the coating operation was the last before placing the article in 25 service. However, it often occurs that after coating the article, it is necessary to work the same, as by bending, rolling, drawing or hammering, and in such case the coating peeled off to a large extent, thus greatly 30 reducing the protective value thereof.

My invention is intended to obviate this disadvantage, it being the objects thereof to provide a method of treating zinc coated materials, which shall prevent the peeling 35 or flaking off of the zinc.

In practicing my invention, I take advantage of the fact that at elevated temperatures zinc is no longer brittle, but becomes malleable, and I have found that between 40 the temperatures 100° C. and 200° C., zinc is sufficiently malleable so that it may be worked. I, therefore, provide a zinc coated article and heat the same to a temperature somewhat above 100° C., whereby the grain 45 structure of the zinc coating is altered and the zinc is rendered malleable. The article is then worked at the elevated temperature, whereby the character of the zinc coating is permanently changed and rendered malleable when cold. The danger of flaking off 50 of the coating is obviated since the zinc by the heating and hot working has been rendered permanently malleable.

A specific example of the operation of

my invention is as follows: In the production of wood strain insulators, I provide a pair of metal caps which are first cleaned and then dipped in molten zinc to provide a hot galvanized coating thereon. The coated caps are then immersed in a bath of 55 acid-free oil heated to a temperature of about 135° C. for a sufficient length of time to allow the caps to attain the temperature of the bath. They are then removed and fitted onto the ends of a treated wood rod 60 and swaged in place.

I have found that I may swage bends in the caps of 45° without any injury whatsoever to the coating. The coating is not only malleable when hot, but also after cooling, and therefore the articles worked in accordance with my invention may afterwards be handled roughly and thrown about without injury to the coating.

Although I have described my invention 75 setting forth a specific embodiment thereof, various changes in the details of my invention may be made within the scope thereof. For instance, my method may be applied to galvanized wire, strap, and the like, which 80 may be subsequently drawn either hot or cold, and also to castings which are subsequently to be stamped or swaged. It is not necessary that the working of the material take place while hot, as good results may be 85 obtained by working the articles after cooling, if the grain structure of the zinc has previously been changed by working the articles hot. These and other changes may 90 be made in my invention without departing 95 from the spirit and scope thereof.

I claim as my invention:

1. A method of treating zinc coated materials which comprises heating the same to a temperature sufficient to change the 95 grain structure of the zinc and then working the material.

2. A method of treating zinc coated materials which comprises heating the same to a temperature above 100° C. and then 100 working the material thereby rendering the coating malleable when cold.

3. A method of treating zinc coated materials which comprises heating the same to a temperature between 100° C. and 200° C., thereby rendering the coating malleable 105 when cold.

4. A method of treating zinc coated ma-

terials which comprises heating the same to a temperature between 100° C. and 200° C. and then working the material.

5. A method of treating zinc coated materials which comprises heating the same to a temperature above 100° C. and then working the material at said temperature.

6. A method of treating zinc coated ma-

terials which comprises heating the same to a temperature between 100° C. and 200° C. 10 and then working the material at said temperatures.

In testimony whereof, I have hereunto subscribed my name this 14th day of December, 1923.

EDGAR CORNELL, JR.